

Patented Dec. 25, 1923.

## UNITED STATES PATENT OFFICE.

GILBERT A. BRAGG, OF SALT LAKE CITY, UTAH, ASSIGNOR TO METALS RECOVERY COMPANY, OF NEW YORK, N. Y., A CORPORATION OF MAINE.

## SELECTIVE FLOTATION OF MINERALS.

No Drawing.

Application filed January 28, 1921. Serial No. 440,759.

To all whom it may concern:

Be it known that I, GILBERT A. BRAGG, a citizen of the United States, residing at Salt Lake City, in the county of Salt Lake, 5 State of Utah, have invented certain new and useful Improvements in Selective Flotation of Minerals; and I do hereby declare the following to be a full, clear, and exact description of the invention, such as will 10 enable others skilled in the art to which it appertains, to make and use the same.

This invention relates to the selective flotation of sulfide minerals, and more particularly to the separation of lead and zinc 15 sulfides by selective flotation.

The invention is based upon the discovery that lead sulfide can be selectively floated from zinc sulfide in a slightly alkaline solution if a small amount of a soluble sulfite, 20 such as sodium sulfite, is present in the ore pulp, and if a suitable flotation agent or agents, operative in a slightly alkaline pulp, are also present.

Where the ore pulp is itself slightly alkaline in reaction, the addition of further amounts of alkaline reagents may be unnecessary. Where, however, the ore pulp is slightly acid, for example, due to oxidation of a small amount of the sulfide mineral, 30 the pulp can be given a slight alkalinity by the addition of a suitable alkaline reagent, such as lime, which I regard as particularly advantageous, although other alkaline reagents can be used, such as sodium sulfide, sodium carbonate or soda ash, caustic soda, etc. The lime can thus be incorporated with the ore pulp during the grinding operation, in such amount as to make the pulp very slightly alkaline.

Various agents for promoting the flotation, which act as flotation agents in a slightly alkaline pulp, can be used. I have found thiocarbanilid particularly advantageous when used together with an agent 40 having good frothing qualities.

The ore can thus be ground with the thiocarbanilid, with sodium sulfite, and with some alkaline substance, such as lime, in sufficient amount to make the pulp very 45 slightly alkaline, and the pulp can then be transferred to a flotation cell, such as a Callow pneumatic cell, and subjected to flotation therein with the addition of a small amount of an agent having good

frothing qualities, such as slightly acidulated aldol.

I have found that sodium sulfite, in such a slightly alkaline pulp, very largely prevents the zinc sulfide from floating, but that the depressing effect upon the lead sulfide is relatively small, so that the lead sulfide will be floated without any appreciable flotation of zinc sulfide. Accordingly, a relatively high grade lead sulfide concentrate can thus be obtained, low in zinc.

After the lead sulfide has thus been selectively floated, the ore pulp is treated to decrease the amount of soluble sulfite remaining therein. For example, the tails from the lead sulfide flotation, can be dewatered to remove a considerable part of the water therefrom, together with a corresponding amount of the sulfite, or the tails can be otherwise treated to decrease the amount of sulfite therein. When the tails are dewatered, for example, to say about 35% solids, a sufficient amount of fresh water can be added to bring the pulp to proper dilution and further amounts of flotation 50 agent or agents added thereto. It is of advantage to add a further amount of alkali, such as sodium carbonate, and also a small amount of copper sulfate to the pulp. So also, a further amount of flotation agent, such as a solution of thiocarbanilid in xylidin, can be added, and the pulp subjected to a further flotation operation and the flotation continued until the zinc sulfide ceases to come over or until the 55 greater part of the zinc sulfide has been floated, and the amount of iron sulfide becomes undesirable in amount as a constituent of the zinc concentrate.

The zinc concentrate thus obtained may 60 contain small and varying amounts of lead sulfide, but when the process is carried out in the manner above described, a further separation of lead from the zinc concentrate can be brought about by tabling to form 65 separate lead and zinc concentrates, and the lead concentrate so obtained can be added to the flotation lead concentrate.

The quantities of reagents used in the practice of the process can be somewhat 70 varied, depending upon the particular ore, etc. Usually only a small amount of soluble sulfite, such as sodium sulfite, will be

necessary, for example, 1 pound of sodium sulfite per ton of ore (that is, figured on the weight of the dry ore and not of the ore pulp). Even such small amounts of sodium sulfite, however, have a marked depressing effect upon the flotation of certain of the sulfides, this depressing effect being most marked on the iron sulfide, and somewhat less marked on the zinc sulfide, while it does not seem to be 10 of important proportions upon lead sulfide. So also, this depressing action seems to be stronger in very slightly alkaline pulps than in pulps which have a decidedly alkaline reaction. Accordingly, only a slight alkaline reaction will usually be desirable. So also, there will ordinarily be no advantage in unnecessarily increasing the amount of sodium sulfite, as only a small amount is required to prevent the flotation of the zinc and iron sulfides, 20 while permitting the flotation of the lead sulfide. I have obtained good results, in the treatment of certain lead-zinc ores, with the use of about 1 pound of lime per ton of ore, about  $\frac{1}{2}$  pound thiocarbanilid per ton of ore and about 1 pound sodium sulfite per ton of ore, adding all of these reagents to the mill and grinding them with the ore; although the amounts of these various reagents are capable of some variation. The nature and 30 amount of the agent added to improve the froth formation is also capable of variation. Acid treated aldon is mentioned as an agent suitable for this purpose in conjunction with thiocarbanilid which has marked selective 35 properties.

After the flotation of the lead sulfide, as above described, the remaining pulp can then be subjected to a dewatering operation to remove as much as possible of the sodium sulfite from the water before attempting to float the zinc. After the pulp has thus been dewatered and again brought to the proper dilution, further amounts of agents promoting the flotation of the zinc sulfide can be 45 added. I have thus found it of advantage to add a small amount of an alkaline substance, such as sodium carbonate, as well as a small amount of copper sulfate, for example, using about 5 pounds of sodium carbonate and 1 pound of copper sulfate per ton of original ore, and thoroughly mixing these reagents with the ore pulp before adding the flotation agent. As a flotation agent for the flotation of the zinc sulfide I have used with 55 advantage a solution of thiocarbanilid in xylidin, containing about 15% thiocarbanilid and 85% xylidin by weight, and using 0.4 pounds of the solution per ton of ore. I have used larger amounts of sodium carbonate and 60 copper sulfate but with the particular ores treated, such larger amounts were not found to be correspondingly more advantageous; while the omission of these two reagents results in the production of a lower grade concentrate.

The process of the present invention is applicable not only to the selective separation of lead and zinc sulfides by flotation, but also to the selective separation of other sulfides from each other. 70

I claim:

1. The method of effecting the selective flotation of sulfide minerals, which comprises subjecting a slightly alkaline pulp, containing a small amount of a soluble sulfite therein, to a flotation operation. 75

2. The method of effecting the selective flotation of lead sulfide from ores containing zinc sulfide, which comprises subjecting a slightly alkaline ore pulp, containing a small amount of a soluble sulfite, to a flotation operation. 80

3. The method of effecting the selective flotation of sulfide minerals, which comprises adding to the mineral pulp a small amount of alkaline substances sufficient to give the pulp a slight alkaline reaction and a small amount of a soluble sulfite, and subjecting the resulting pulp to a flotation operation. 85

4. The method of effecting the selective flotation of lead sulfide from ores containing zinc sulfide which comprises adding to the ore pulp a small amount of an alkaline substance to give the pulp a slight alkaline reaction, adding a small amount of a soluble sulfite, together with a suitable flotation agent, and subjecting the resulting pulp to a flotation operation. 90

5. The method of effecting the selective flotation of lead sulfide from ores containing zinc sulfide, which comprises adding to the ore pulp a small amount of an alkaline substance to give the pulp a slight alkaline reaction, together with a small amount of a soluble sulfite, a small amount of thiocarbanilid and an agent having good frothing qualities, and subjecting the resulting pulp to a flotation operation. 100

6. The method of effecting the selective flotation of sulfide minerals, which comprises subjecting a slightly alkaline pulp containing a small amount of a soluble sulfite therein to a flotation operation to remove certain of the sulfides, reducing the amount of soluble sulfide remaining in the pulp and subjecting the pulp to a further flotation operation for the flotation of other sulfides. 110

7. The method of effecting the selective flotation of lead and zinc sulfides which comprises subjecting a slightly alkaline pulp containing a small amount of a soluble sulfite to a flotation operation for the production of a lead sulfide concentrate, decreasing the amount of soluble sulfite in the remaining ore pulp to an amount permitting flotation of zinc sulfide, and subjecting the ore pulp to a further flotation operation. 120

8. The method of effecting the selective flotation of lead and zinc sulfides, which comprises subjecting a slightly alkaline ore pulp containing a small amount of a soluble sulfite to a flotation operation for the production of a lead concentrate, treating the remaining pulp to reduce the amount of soluble sulfite therein to permit flotation of zinc sulfide, adding a further amount of alkali and of a flotation agent and subjecting the pulp to a further flotation for the production of a zinc concentrate.

9. The method of effecting the selective flotation of lead and zinc sulfides, which comprises subjecting a slightly alkaline ore pulp in the presence of a soluble sulfite to a flotation operation for the production of a lead sulfide concentrate, removing a considerable portion of the sulfite from the ore pulp, adding thereto a small amount of an alkaline substance and a small amount of copper sulfate together with a flotation agent and subjecting the pulp to a further flotation operation for the treatment of a zinc concentrate.

10. The method of effecting the selective flotation of lead and zinc sulfides, which comprises adding to the ore pulp a small amount of an alkaline substance to give the

pulp a slight alkaline reaction, adding a small amount of a soluble sulfite, a small amount of thiocarbanilid and a small amount of a substance having good frothing qualities, subjecting the pulp to a flotation operation for the production of a lead concentrate, treating the remaining pulp to reduce the amount of soluble sulfite therein, adding a further amount of an alkaline substance and of a flotation agent thereto, and subjecting the pulp to a further flotation operation for the production of a zinc concentrate.

11. The method of effecting the separation of lead and zinc sulfide, which comprises subjecting a slightly alkaline ore pulp containing them and containing a small amount of a soluble sulfite to a flotation operation for the production of a lead concentrate, decreasing the amount of soluble sulfite in the remaining pulp to permit the flotation of zinc sulfide, subjecting the pulp to a further flotation operation for the production of a zinc concentrate, and subjecting the zinc concentrate to a tabling operation to effect the separation of small amounts of lead sulfide therefrom.

In testimony whereof I affix my signature.  
GILBERT A. BRAGG.